# EUROPEAN PATENT SPECIFICATION

(11) **EP 4 298 258 B1**
(45) Date of publication and mention of the grant of the patent: **14.01.2026**
(21) Application number: 22704766.9
(22) Date of filing: 10.02.2022
(51) Int. Cl.: C22C 21/00, C22C 21/06, C22C 21/08, C22F 1/047

(54) **DURABLE ALUMINIUM ALLOY SHEET FOR DECORATIVE APPLICATIONS**
LANGLEBIGES ALUMINIUM-LEGIERUNGSBLECH FÜR DEKORATIVE ANWENDUNGEN
TOLE MINCE DURABLE EN ALLIAGE D'ALUMINIUM POUR APPLICATIONS DÉCORATIVES

(30) Priority: 26.02.2021 EP 21159556
(43) Date of publication of application: 03.01.2024
(73) Proprietor: Constellium Rolled Products Singen GmbH & Co.KG, 78224 Singen (DE)
(72) Inventor: LAE, Emilie, 38430 SAINT JEAN DE MOIRANS (FR); SIGLI, Christophe, 38000 GRENOBLE (FR); SEEMÜLLER, Christoph, 78462 KONSTANZ (DE)
(74) Representative: Constellium - Propriété Industrielle
(86) International application number: PCT/EP2022/053220
(87) International publication number: WO 2022/179856

(56) References cited:
- WO-A1-2016/039215
- CN-A- 102 703 776
- CN-A- 108 330 417

## Description

### Field of the invention

The invention relates to the field of decorative parts made of aluminium alloys which are formable. These parts are coated before forming for decorative purposes and/or to be durable. The alloy after the curing of the coating must be hard enough to present a good dent or scratch resistance.

The invention relates more particularly to aluminium alloy sheets of the AA3XXX and AA5xxx series with a composition and manufacturing process that are particularly suitable for this type of application and offering,

### State of the art

Aluminium alloys are commonly used in the manufacturing of decorative parts, particularly for the automotive industry, but also in the household appliance and medical device industries, in competition with wood, steel and plastics. These parts are generally coated, typically with a varnish or a paint.

In the case of the automotive industry, interior decorative elements are produced, for example for high-usage door handles, gearbox trims, light-resistant and shockproof trim elements for the center console, trims and/or panels on the dashboard and/or doors, capacitive function elements and exterior elements are also produced such as, in particular, the window surrounds, body side or door trim strips, beltlines, tailgate trim strips, radiator grille trim, bumper piping, hubcaps, wheel hub cover....

Two types of products are currently available on the market: extruded profiles and shaped sheets.

The predominant alloy types used for sheets are AA 1XXX, AA3XXX, AA5XXX and 8XXX alloys. AA5005 aluminium alloy rolled products with different heat treatment states are widely used in conductors, kitchenware, dashboards, architectural decorations, building materials, vehicle interior and exterior materials.

WO/2014/203077 relates to a method for manufacturing an outer moulding ring of a motor vehicle, in particular such as a window frame or body shell moulding, made of an aluminium alloy, by shaping and polishing a sheet or strip made by continuous vertical casting of a high-purity alloy sheet of series AA5xxx.

Several patents disclose Al-Mn-Mg alloys, mainly for packaging applications: EP0504077 relates to Al-based alloys intended for deep drawing and/or drawing and exhibiting high mechanical strength characteristics as well as good isotropy (low distortion wedge content) and good cold processability having the following compositions by weight (%): Fe ≦ 0.25 - Si ≦ 0.25 - Mn from 0.8 to 1.6 - Mg from 0.7 to 2.5 - Cu from 0.20 to 0.6 - Cr from 0 to 0.35 - Ti from 0 to 0.1 - V from 0 to 0.1 - others each ≦ 0,05, total ≦ 0,15, remainder Al.

WO/2018/143376 relates to an aluminium alloy sheet which contains 0.05-0.60 mass% of Si, 0.05-0.80 mass% of Fe, 0.05-0.25 mass% of Cu, 0.80-1.50 mass% of Mn, 0.80-1.50 mass% of Mg, Al, and incidental impurities.

WO2015140833 relates to an aluminium alloy for can bodies containing Si: 0.10-0.60 mass%, Fe: 0.10-0.80%, Cu: 0.05-0.25%, Mn: 0.80-1.50%, Mg: 0.80-1.30% and the remainder being obtained from Al and unavoidable impurities.

WO/2016/149061 relates to aluminium alloys for making packaging products such as bottles and cans comprising 0.1-1.6 wt. % Mn, 0.1-3 wt. % Mg, 0.1-1.5 wt. % Cu, 0.2-0.7 wt. % Fe, 0.10-0.6 wt. % Si, up to 0.3 wt. % Cr, up to 0.6 wt. % Zn, up to 0.2 wt. % Ti, 0.05 wt. % for each trace element, <0.15 wt. % for total trace elements and remainder Al.

WO/2016/100800 relates to compositions and methods comprising aluminium alloy system useful for aluminium bottle applications comprising about 0.15-0.50 % Si, 0.35-0.65 % Fe, 0.05-0.30 % Cu, 0.60-1.10 % Mn, 0.80-1.30 % Mg, 0.000-0.0080 % Cr, 0.000-0.500 % Zn, 0.000-0.080 % Ti, up to 0.15 % of impurities, with the remainder as Al. CN102703776 relates to an aluminum alloy substrate for a light-emitting diode (LED) television and a production method for the aluminum alloy substrate. The substrate comprises the following components in percentage by mass: 0.20 to 0.50 percent of Si, 0.30 to 0.70 percent of Fe, less than or equal to 0.25 percent of Cu, 0.8 to 1.0 percent of Mn, 1.10 to 1.25 percent of Mg, 0.12 to 0.30 percent of Cr, less than or equal to 0.25 percent of Ti, less than 0.10 percent of Zn and the balance of Al. There are four main requirements for these products: good formability, in order to provide the desired shape, nice surface aspect without surface defects generated by forming such as Portevin Le Chatelier bands, Lüders bands or orange peel, sufficient durability such as corrosion resistance and scratch resistance. Current alloys used for such applications (such as 5005, 8014 or 1050) typically have the requested formability, corrosion resistance and surface aspect but they may however undergo scratches /dents. A product with an improved resistance to scratches or dents is requested by the industry, without degrading any of the other properties.

### The problem

The invention aims to provide sheets made of aluminium alloys that are particularly suitable to make decorative parts and offer a high scratch resistance, with simultaneously being formable, corrosion resistant and providing a nice surface aspect.

### Subject of the invention

The invention is as set forth in the appended claims.

A first subject of the invention is a sheet made of an aluminium alloy comprising, by weight %
Mg : 0.8 - 1.3,
Mn : 0.8 - 1.2,
Cu: 0.05 - 0.30,
Cr : 0.05 - 0.30,
Fe : ≤ 0.4,
Si : ≤ 0.3,
Zn : ≤ 0.25,
Ti : ≤ 0.15,
impurities < 0.05 each and < 0.15 total, remainder aluminium, wherein the conventional yield strength YTS in the longitudinal direction is at least 130 MPa and the elongation break A% in the longitudinal direction is at least 13%.

Another subject of the invention is a method to make a sheet according to the invention wherein,
(a) a slab is cast of an aluminium alloy comprising, by weight %
   Mg : 0.8 - 1.3,
   Mn : 0.8 - 1.2,
   Cu: 0.05 - 0.30,
   Cr : 0.05 - 0.30,
   Fe : ≤ 0.4,
   Si : ≤ 0.3,
   Zn : ≤ 0.25,
   Ti : ≤ 0.15,
   impurities < 0.05 each and < 0.15 total, remainder aluminium,
(b) the slab is homogenized at a temperature of at least 550 °C,
(c) the homogenized slab is hot rolled to an intermediate rolled product having a thickness from 3 to 10 mm,
(d) the intermediate rolled product is cold rolled into a sheet, optionally with an intermediate annealing during cold rolling,
(e) the sheet is annealed at a temperature from 300°C to 400 °C and undergoes tension leveling with a stretching of at least 1.8%.

Yet another subject of the invention is the use of a sheet according to the invention to make a coated decorative part preferably a decorative part for an automobile, or a household appliance or a medical device.

### Description of the invention

Unless otherwise indicated, all indications concerning the chemical composition of alloys are expressed as a percentage by weight based on the total weight of the alloy. The expression 1.4 Cu means that the copper content expressed in % by weight is multiplied by 1.4. The designation of the alloys is made in accordance with the regulations of The Aluminium Association, known to those skilled in the art.

The static mechanical properties in tension, in other words the ultimate tensile strength UTS, the conventional yield strength at 0.2 % elongation TYS, and the elongation at break A%, are determined by a tensile test according to standard NF EN ISO 6892-1. The elongation (A%) at break was measured using a 50 mm base extensometer and is reported under A50. Scratch resistance was measured according to the method described in the example.

Unless stated otherwise, the definitions of standard EN 12258 (2012) apply. A sheet is a rolled product with a rectangular cross section, the uniform thickness of which is between 0.20 mm and 6 mm. In the context of the invention, a sheet is not a clad sheet. A preferred thickness of the sheet of the invention is from 0.35 mm to 1.5 mm and more preferably from 0.50 mm to 1.0 mm.

The inventors have found a sheet composition which solves the problem. In particular, with the simultaneous addition of Cu and Cr to an Al-Mg-Mn alloy, the sheet of the invention provides higher scratch resistance with similar formability and corrosion resistance than the known products.

The present inventors had first considered to use a high Mg content such as 1.8 wt.% in order to improve scratch resistance, however the products obtained had surface defects related to Lüders bands / Portevin-Le Chatelier bands observed during forming. In order to avoid these bands, the magnesium content has to be at most 1.3 wt.%. A minimum Mg content of 0.8 wt.% is needed to obtain sufficient strength and scratch resistance. Preferably the minimum Mg content is 0.9 wt.%. Preferably the maximum Mg content is 1.2 wt.% and more preferably 1.1 wt.%. In a preferred embodiment by wt.%, Mg : 0,9 - 1.1.

Mn is used to improve strength and scratch resistance. The Mn content is from 0.8 to 1.2 wt.%. Preferably the minimum Mn content is 0.85 wt.%, more preferably 0.90 wt.% and preferentially 0.95 wt.%. Preferably the maximum Mn content is 1.15 wt.% and more preferably 1.10 wt.% and preferentially 1.05 wt.%. In a preferred embodiment by wt.%, Mn : 0.85 - 1.15 and preferably Mn : 0.95 - 1.05.

Cu is added to improve strength and scratch resistance. The Cu content is from 0.05 to 0.30 wt.%. Preferably the minimum Cu content is 0.10 wt.%, more preferably 0.15 wt.%. Preferably the maximum Cu content is 0.25 wt.% and more preferably 0.20 wt.%. In a preferred embodiment by wt.%, Cu : 0.10 - 0.25 and preferably Cu : 0.15 - 0.20.

Cr is added to improve strength and scratch resistance. The Cr content is from 0.05 to 0.30 wt.%. Preferably the minimum Cr content is 0.10 wt.%, more preferably 0.15 wt.%. Preferably the maximum Cr content is 0.27 wt.% and more preferably 0.25 wt.%. In a preferred embodiment by wt. % Cr : 0.10 - 0.30 and preferably Cr : 0.15 - 0.25.

Fe and Si have to be limited to a maximum of 0.4 wt.% and 0.3 wt.%, respectively, to obtain the desired formability. A minimum content is however beneficial for surface aspects by limiting, for example, orange peel aspect on formed parts. The inventors believe that Fe and Si additions increase the Particle Stimulated Nucleation effect during recrystallization compared to a purer chemistry, which leads to smaller grains and limits the orange peel on formed parts. Preferably the minimum Fe content is 0.15 wt.%, more preferably 0.20 wt.%. Preferably the maximum Fe content is 0.35 wt.% and more preferably 0.30 wt.%. In a preferred embodiment by wt.%, Fe : 0.15 - 0.35 and/or Si : 0.10 - 0.25.

Preferably the minimum Si content is 0.10 wt.%, more preferably 0.15 wt.% and even more preferably 0.18 wt.%. Preferably the maximum Si content is 0.25 wt.% and more preferably 0.23 wt.%.

With the selected preferred Fe and Si contents recyclability of the alloy is quite satisfactory.

The Zn content is limited to a maximum of 0.25 wt.%. Further limiting the zinc content usually degrades recyclability. In an embodiment the Zn content is at least 0.01 wt.%. In another embodiment the Zn content is however limited to an impurity level of less than 0.01 wt.% to improve surface aspect.

The Ti content is limited to a maximum of 0.15 wt.%. Ti may be added to improve grain size control, in particular during casting. In an embodiment the Ti content is at least 0.01 wt.%. Preferably the maximum Ti content is 0.10 wt.% and more preferably 0.05 wt.%. Other elements are impurities whose content is less than 0.05 wt.% each and 0.15 wt.% total.

The method to make a sheet according to the invention comprises casting a slab with a composition according to the invention, homogenizing, hot and cold rolling the slab, annealing and tension leveling.

The slab is homogenized at a temperature of at least 550 °C, preferably of at least 575 °C. The maximum homogenizing temperature is defined to avoid incipient melting, it is typically 630 °C or 620 °C. Preferably, the homogenization is carried out during at least one hour and at most 72 hours. Before or after homogenization, the slab is usually scalped. The homogenized slab is then hot rolled to an intermediate rolled product having a thickness from 3 to 10 mm. Preferably the initial hot rolling temperature is at least 430 °C. The intermediate rolled product is then cold rolled into a sheet, optionally with an intermediate annealing during cold rolling. In an embodiment the intermediate rolled product is first cold rolled to a first thickness between 1.5 and 8.0 mm, then annealed at a temperature from 300 °C to 450 °C and then cold rolled to a second thickness between 0.20 mm and 6 mm. In another embodiment, the intermediate rolled product is directly cold rolled into a sheet with a thickness between 0.20 mm and 6 mm.

The sheet is then annealed at a temperature from 300 °C to 450 °C. The annealing is designed to obtain full recrystallization. The temper after annealing is named O-temper. Finally, the sheet undergoes tension leveling with a stretching of at least 1.8 %.

Tension leveling is needed to improve flatness of the product. Advantageously, a minimum stretching during tension leveling of 2 %, is performed in order to improve the yield strength after curing of the coating, typically of 1 to 10 minutes at 150 to 230 °C. In order to prevent surface defects and preserve good formability a maximum stretching of 3.5 %, more preferably 3 %, during tension leveling is performed. The sheets of the invention have preferably, after tension leveling a TYS in the longitudinal direction of at least 130 MPa and A% of at least 13% and preferably of at least 16 % and after further thermal treatment of 4 minutes at 195 °C, typically corresponding to curing of the coating, a TYS in the longitudinal direction of at least 110 MPa and A% of at least 16 %. The sheets according to the invention are preferably used to make a coated decorative part, preferably for an automobile, or a household appliance or a medical device. Preferably they are used to make an automobile interior finishing element selected in the list consisting of a door handle, a gearbox trim, a trim element for a center console, a trim for a dashboard, a panel for a dashboard, a trim for a door, a panel for a door and a capacitive function element or an automobile exterior element selected in the list consisting of a window surrounds, a body side or door trim strip, a tailgate trim strip, a radiator grille trim, wheel hub cover, a beltline and a bumper piping.

The details of the invention will be understood better with the help of the example below, which is not, however, restrictive in its scope.

### Example

The alloys disclosed in Table 1 where cast in the form of small ingots of dimension 70 mm x 190 mm x 1500 mm. Alloy C is according to the invention.

**Table 1: Composition in wt.%**

| **Alloy** | **Si %** | **Fe %** | **Cu %** | **Mn %** | **Mg %** | **Cr %** | **Zn** | **Ti** |
|---|---|---|---|---|---|---|---|---|
| **A** | 0.11 | 0.20 | 0.17 | 0.97 | 1.1 | < 0.01 | <0.01 | 0.01 |
| **B** | 0.10 | 0.19 | < 0.01 | 1.02 | 1.3 | 0.18 | <0.01 | 0.01 |
| **C** | 0.11 | 0.20 | 0.16 | 1.00 | 1.1 | 0.21 | <0.01 | 0.01 |

The ingots were scalped and homogenized 3 hours at 600 °C. The ingots were hot rolled with a starting temperature above 500 °C down to a thickness of 7.6 mm and cold rolled to a thickness of 2.5 mm. An intermediate annealing of 1 hour at 340 °C was carried out and the cold rolling was continued to sheets with a thickness of 0.76 mm. The sheets were annealed 1 hour at 340 °C to obtain a fully recrystallized grain structure. The sheets were then tension-levelled with a stretching of 2.5 % in the rolling direction.

In order to obtain representative mechanical properties of the finished part, which is formed and coated, a coating curing simulation of 4 min at 195 °C was carried out. Mechanical properties characterized in the longitudinal direction L are provided in Table 2.

**Table 2: Mechanical properties of the sheets**

| | **Recrystallized** | **+ stretching 2.5 % by tension leveling** | | **+ 4 min at 195°C** | | | |
|---|---|---|---|---|---|---|---|
| **Alloy** | TYS (MPa) | TYS (MPa) | A50 (%) | TYS (MPa) | UTS (MPa) | TYS/UTS (-) | A50 (%) |
| **A** | 65 | 126 | 17.2 | 105 | 182 | 0.57 | 15.8 |
| **B** | 64 | 127 | 18.2 | 102 | 177 | 0.58 | 18.3 |
| **C** | 68 | 135 | 17.8 | 113 | 191 | 0.59 | 17.0 |

All samples were also coated with the same varnish thickness and scratch resistance was tested with a scratch hardness tester (Erichsen Model 435 pen).

The test range used is 0 to 20N (range 3 of the apparatus). The test wheel used is the provided steel disc. The hardness tester is placed perpendicularly onto the surface to be tested and is pressed down so that the guide wheels touch the surface. In this way the preset force acting upon the test disc is fully effective on the test surface. The instrument is then moved, the wheel being over the specimen to be tested.

The scratch resistance is related to maximum force at which the test body does not leave any trace on the test surface. The results are presented in Table 3 in a comparative manner compared to a typical requirement "+" slightly above requirement, "++" significantly above requirement.

**Table 3: Scratch resistance of the sheets**

| **Alloy** | **scratch resistance** |
|---|---|
| **A** | + |
| **B** | + |
| **C** | ++ |

With the composition according to the invention, an improved scratch resistance is obtained, without degrading elongation before or after the curing.

### Example 2

In this example, a product according to the invention of industrial dimensions was obtained. The alloy disclosed in Table 4 was cast in the form of an ingots of industrial dimension.

**Table 4. Composition in wt.%**

| **Alloy** | **Si %** | **Fe %** | **Cu %** | **Mn %** | **Mg %** | **Cr %** | **Zn** | **Ti** |
|---|---|---|---|---|---|---|---|---|
| **D** | 0.20 | 0.24 | 0.16 | 0.95 | 1.0 | 0.18 | 0.006 | 0.03 |

The ingots was scalped and homogenized 3 hours at 600 °C. The ingot was hot rolled with a starting temperature above 500 °C down to a thickness of 7.6 mm and directly cold rolled to a sheet with a thickness of 0.76 mm. The sheet was annealed 1 hour at 340 °C to obtain a fully recrystallized grain structure. Finally, tension leveling of the sheet was carried out with a 2.5% stretch.

Mechanical properties characterized in the rolling direction L are provided in Table 5.

**Table 5: Mechanical properties of the sheets**

| | **Recrystallized** | **+ stretching 2.5 % by tension leveling** | |
|---|---|---|---|
| **Reference** | **YS (MPa)** | **YS (MPa)** | A50 (%) |
| **D** | 74 | 130 | 13.5 |

The scratch resistance of the sheets was evaluated in the same way as in example 1. The result was ++.

## Claims

1. Sheet made of an aluminium alloy comprising, by weight %
Mg : 0.8 - 1.3,
Mn : 0.8 - 1.2,
Cu: 0.05 - 0.30,
Cr : 0.05 - 0.30,
Fe : ≤ 0.4,
Si : ≤ 0.3,
Zn : ≤ 0.25,
Ti : ≤ 0.15,
impurities < 0.05 each and < 0.15 total, remainder aluminium, wherein the conventional yield strength, TYS, in the longitudinal direction is at least 130 MPa and the elongation at break, A%, in the longitudinal direction is at least 13%, determined by a tensile test according to standard NF EN ISO 6892-1 and A% was measured using a 50 mm base extensometer.

2. Sheet according to claim 1 comprising by wt. % Cr : 0.10 - 0.30 and preferably Cr : 0.15 - 0.25.

3. Sheet according to claim 1 or claim 2 comprising, by wt.%, Fe : 0.15 - 0.35 and/or Si : 0.10 - 0.25.

4. Sheet according to anyone of claims 1 to 3 comprising, by wt.%, Mg : 0.9 - 1.1.

5. Sheet according to anyone of claims 1 to 4 comprising, by wt.%, Mn : 0.85 - 1.15 and preferably Mn : 0.95 - 1.05.

6. Sheet according to anyone of claims 1 to 5 comprising, by wt.%, Cu : 0.10 - 0.25 and preferably Cu : 0.15 - 0.20.

7. Sheet according to anyone of claims 1 to 6 wherein, after a thermal treatment of 4 min at 195 °C TYS in the longitudinal direction is at least 110 MPa and A% in the longitudinal direction is at least 16%.

8. Method to make a sheet according to anyone of claims 1 to 7 wherein,
(a) a slab is cast of an aluminium alloy comprising, by weight %
Mg : 0.8 - 1.3,
Mn : 0.8 - 1.2,
Cu: 0.05 - 0.30,
Cr : 0.05 - 0.30,
Fe : ≤ 0.4,
Si : ≤ 0.3,
Zn : ≤ 0.25,
Ti : ≤ 0.15,
impurities < 0.05 each and < 0.15 total, remainder aluminium,
(b) the slab is homogenized at a temperature of at least 550 °C,
(c) the homogenized slab is hot rolled to an intermediate rolled product having a thickness from 3 to 10 mm,
(d) the intermediate rolled product is cold rolled into a sheet, optionally with an intermediate annealing during cold rolling,
(e) the sheet is annealed at a temperature from 300°C to 400 °C and undergoes tension leveling with a stretching of at least 1.8%.

9. Use of a sheet according to anyone of claims 1 to 7 to make a coated decorative part preferably a decorative part for an automobile, or a household appliance or a medical device.

10. Use according to claim 9 to make an automobile interior finishing element selected in the list consisting of a door handle, a gearbox trim, a trim element for a center console, a trim for a dashboard, a panel for a dashboard, a trim for a door, a panel for a door and a capacitive function element or an automobile exterior element selected in the list consisting of a window surrounds, a body side or door trim strip, a tailgate trim strip, a radiator grille trim, wheel hub cover, a beltline and a bumper piping.

## Patentansprüche

1. Blech aus einer Aluminiumlegierung, umfassend, in Gewichtsprozent,
Mg: 0,8 - 1,3,
Mn: 0,8 - 1,2,
Cu: 0,05 - 0,30,
Cr: 0,05 - 0,30,
Fe: ≤ 0,4,
Si: ≤ 0,3,
Zn: ≤ 0,25,
Ti: ≤ 0,15,
Verunreinigungen je < 0,05 und insgesamt < 0,15, Rest Aluminium, wobei die konventionelle Streckgrenze, TYS, in Längsrichtung mindestens 130 MPa beträgt und der Dehnungsbruch, A %, in Längsrichtung mindestens 13 % beträgt, ermittelt durch eine Zugprüfung gemäß der Norm NF EN ISO 6892-1, und A% wurde mit einem 50-mm-Basis-Dehnmessgerät gemessen.

2. Blech nach Anspruch 1, umfassend, in Gew.-%, Cr: 0,10 - 0,30 und vorzugsweise Cr: 0,15 - 0,25.

3. Blech nach Anspruch 1 oder Anspruch 2, umfassend, in Gew.-%, Fe: 0,15 - 0,35 und/oder Si: 0,10 - 0,25.

4. Blech nach einem der Ansprüche 1 bis 3, umfassend, in Gew.-%, Mg: 0,9 - 1,1.

5. Blech nach einem der Ansprüche 1 bis 4, umfassend, in Gew.-%, Mn: 0,85 - 1,15 und vorzugsweise Mn: 0,95 - 1,05.

6. Blech nach einem der Ansprüche 1 bis 5, umfassend, in Gew.-%, Cu: 0,10 - 0,25 und vorzugsweise Cu: 0,15 - 0,20.

7. Blech nach einem der Ansprüche 1 bis 6, wobei nach einer Wärmebehandlung von 4 min bei 195 °C TYS in Längsrichtung mindestens 110 MPa beträgt und A % in Längsrichtung mindestens 16 % beträgt.

8. Verfahren zum Herstellen eines Blechs nach einem der Ansprüche 1 bis 7, wobei
a) eine Platte aus einer Aluminiumlegierung gegossen wird, umfassend, in Gewichtsprozent,
Mg: 0,8 - 1,3,
Mn: 0,8 - 1,2,
Cu: 0,05 - 0,30,
Cr: 0,05 - 0,30,
Fe: ≤ 0,4,
Si: ≤ 0,3,
Zn: ≤ 0,25,
Ti: ≤ 0,15,
Verunreinigungen je < 0,05 und insgesamt < 0,15, Rest Aluminium,
b) die Platte bei einer Temperatur von mindestens 550 °C homogenisiert wird,
c) die homogenisierte Platte zu einem Zwischenwalzprodukt mit einer Dicke von 3 bis 10 mm warmgewalzt wird,
d) das Zwischenwalzprodukt zu einem Blech kaltgewalzt wird, optional mit einer Zwischenglühung während des Kaltwalzens,
e) das Blech bei einer Temperatur von 300 °C bis 400 °C geglüht und einer Spannungsausgleichung mit einer Dehnung von mindestens 1,8 % unterzogen wird.

9. Verwendung eines Blechs nach einem der Ansprüche 1 bis 7 zum Herstellen eines beschichteten Dekorationsteils, vorzugsweise eines Dekorationsteils für ein Automobil oder ein Haushaltsgerät oder ein Medizinprodukt.

10. Verwendung nach Anspruch 9 zum Herstellen eines Innenausstattungselements für Kraftfahrzeuge, ausgewählt aus der Liste, bestehend aus einem Türgriff, einer Getriebeverkleidung, einem Verkleidungselement für eine Mittelkonsole, einer Verkleidung für ein Armaturenbrett, eine Blende für ein Armaturenbrett, einer Verkleidung für eine Tür, einer Blende für eine Tür und einem kapazitivem Funktionselement, oder eines Außenelements für Kraftfahrzeuge, ausgewählt aus der Liste, bestehend aus einem Fensterrahmen, einer Karosserieseiten- oder Türverkleidungsleiste, einer Heckklappenverkleidungsleiste, einer Kühlergrillverkleidung, einer Radnabenabdeckung, einer Seitenzierleiste und eine Stossfängerverkleidung.

## Revendications

1. Tôle en alliage d'aluminium comprenant, en % en poids
Mg : 0,8 - 1,3,
Mn : 0,8 - 1,2,
Cu : 0,05 - 0,30,
Cr : 0,05 - 0,30,
Fe : ≤ 0,4,
Si : ≤ 0,3,
Zn : ≤ 0,25,
Ti : ≤ 0,15,
impuretés < 0,05 chacune et < 0,15 au total, le reste étant de l'aluminium, dans laquelle la limite d'élasticité conventionnelle, TYS, dans le sens longitudinal est d'au moins 130 MPa et l'allongement à la rupture, A %, dans le sens longitudinal est d'au moins 13 %, déterminée par un essai de traction selon la norme NF EN ISO 6892-1 et A % a été mesuré à l'aide d'un extensomètre sur base de 50 mm.

2. Tôle selon la revendication 1 comprenant, en % en poids, Cr : 0,10 - 0,30 et de préférence Cr : 0,15 - 0,25.

3. Tôle selon la revendication 1 ou la revendication 2 comprenant, en % en poids, Fe : 0,15 - 0,35 et/ou Si : 0,10 - 0,25.

4. Tôle selon l'une quelconque des revendications 1 à 3 comprenant, en % en poids, Mg : 0,9 - 1,1.

5. Tôle selon l'une quelconque des revendications 1 à 4 comprenant, en % en poids, Mn : 0,85 - 1,15 et de préférence Mn : 0,95 - 1,05.

6. Tôle selon l'une quelconque des revendications 1 à 5 comprenant, en % en poids, Cu : 0,10 - 0,25 et de préférence Cu : 0,15 - 0,20.

7. Tôle selon l'une quelconque des revendications 1 à 6 dans laquelle, après un traitement thermique de 4 min à 195 °C, TYS dans le sens longitudinal est d'au moins 110 MPa et A % dans le sens longitudinal est d'au moins 16 %.

8. Procédé de fabrication d'une tôle selon l'une quelconque des revendications 1 à 7 dans lequel,
(a) une brame est coulée en alliage d'aluminium comprenant, en % en poids
Mg : 0,8 - 1,3,
Mn : 0,8 - 1,2,
Cu : 0,05 - 0,30,
Cr : 0,05 - 0,30,
Fe : ≤ 0,4,
Si : ≤ 0,3,
Zn : ≤ 0,25,
Ti : ≤ 0,15,
impuretés < 0,05 chacune et < 0,15 au total, le reste étant de l'aluminium,
(b) la brame est homogénéisée à une température d'au moins 550 °C,
(c) la brame homogénéisée est laminée à chaud jusqu'à un produit laminé intermédiaire ayant une épaisseur de 3 à 10 mm,
(d) le produit laminé intermédiaire est laminé à froid en une tôle, éventuellement avec un recuit intermédiaire pendant le laminage à froid,
(e) la tôle est recuite à une température de 300 °C à 400 °C et soumise à un planage par étirage avec un étirement d'au moins 1,8 %.

9. Utilisation d'une tôle selon l'une quelconque des revendications 1 à 7 pour fabriquer une pièce décorative revêtue, de préférence une pièce décorative pour un véhicule automobile, ou un appareil électroménager ou un dispositif médical.

10. Utilisation selon la revendication 9 pour fabriquer un élément de finition intérieur automobile sélectionné dans la liste consistant en une poignée de porte, une graniture de boîte de vitesses, **un** élément d'habillage pour une console centrale, un habillage pour un tableau de bord, un panneau pour un tableau de bord, **un** habillage pour une porte, un panneau pour une porte et **un** élément à fonction capacitive ou un élément extérieur automobile sélectionné dans la liste consistant en **un** encadrement de vitre, un bande de flanc de carrosserie ou une baguette décorative de porte, une baguette décorative de hayon, une calandre, un enjoliveur, une ligne de ceinture et un pare-chocs tube.
